

Patented Feb. 29, 1944

2,343,125

# UNITED STATES PATENT OFFICE

2,343,125

## LUBRICATING OIL COMPOSITION

Robert G. Larsen and Frederic A. Armfield, Berkeley, Calif., assignors to Shell Development Company, San Francisco, Calif., a corporation of Delaware

No Drawing. Application July 29, 1941,  
Serial No. 404,509

13 Claims. (Cl. 252—55)

This invention deals with lubricants which are relatively stable under oxidation conditions and is more particularly concerned with mineral lubricating oils to which a preoxidized alkylated aromatic component has been added.

Lubricating, transformer, turbine, and other refined relatively heavy mineral oils suffer a marked deterioration in use and when exposed to air at elevated temperatures. Generally, such petroleum oils when in use darken in color and eventually may become saturated with and deposit a finely-divided oil-insoluble carbonaceous material, commonly known as sludge. Under some conditions they may deposit a varnish on hot metal surfaces. Such oils, in addition, develop an acidity after some period of use, particularly when used under high temperature conditions. It has been established that the formation of acids is due to oxidation, and it is thought that the formation of sludge may be due to polymerization and/or oxidation. Varnish formation is believed to be caused by similar reactions. The rapidity of this deterioration varies with various oils and depends upon their sources and degree of refinement as well as on the conditions to which they are exposed. In many cases the deterioration appears to be an autocatalytic phenomenon in that products of the reaction serve to speed up or catalyze the further deterioration of the oil itself.

There are two types of addition agents which, when added to lubricating, etc. oils, prevent oil deterioration through oxidation. The type known as inhibitors are themselves oxidized and rendered useless for protecting the oil further. Oxidation of inhibited oils is therefore very slow at first and then experiences a break to a marked and sudden increase. On the other hand, the type known as retarders are oxidized readily at first but increase their inhibiting powers as oxidation proceeds. Oxidation of oils containing retarders is therefore initially fast and then approaches an extended stage where oxidation proceeds at a rather uniform, greatly reduced speed.

Inhibitor type compounds are best illustrated by the alkylated phenols, while retarder type compounds are illustrated by certain aromatic sulfur compounds such as dibenzyl disulfide. The disadvantage of the former is that they are soon oxidized and lose their effectiveness, while the disadvantage of the latter is that apparently they foster sludge formation.

Where certain selected stable aromatics act as inhibitors, retarders, or a combination of both, and render lubricating oils in which they are dissolved in small quantities less susceptible to attack by oxygen, the oxidation of the unstable constituents of the refined oil proceeds competitively, or at a slower rate than oxidation of the aromatic. Some aromatics such as alkylated naphthalene are so stable that they do not oxidize ap-

preciable in the presence of the unstable constituents found in refined oils and therefore have little, if any, oxidation-inhibiting effect.

Now it has been discovered that the addition of products obtained by oxidizing stable alkyl-substituted aromatic hydrocarbons, free from polar radicals and having more than one condensed ring, to mineral lubricating oils in suitable small quantities, produces lubricating oils of improved oxidation stability.

The stable alkylated multi-nuclear aromatic hydrocarbons which we may oxidize to form our useful anti-oxidant are either (1) the pure compounds such as naphthalenes or preferably alkylated naphthalenes having one or more alkyl groups attached to the naphthalene nucleus, e. g., naphthalene, alpha- or beta-methyl, -ethyl, -isopropyl, -isopropyl; primary-, secondary-, or tertiary-butyl, -amyl, etc., naphthalenes; 1-2, 1-4, 1-5, 1-7, 1-8, 2-3, 2-5, 2-6, 2-7 di-methyl, di-ethyl, methyl-ethyl, methyl-propyl, methyl-isopropyl, di-isopropyl, methyl-butyl, isopropyl-tertiary-butyl, di-primary, -secondary, or tertiary butyl, di-primary, secondary or tertiary amyl, etc., tri, tetra, penta, etc., alkyl naphthalenes or corresponding alkylated anthracenes, phenanthrenes, and other highly condensed aromatics, etc.; or (2) highly aromatic relatively high-boiling fractions of coking cycle stocks, a substantial portion of which boils above 240° C., such as are obtained by operating a liquid phase cracking unit under conditions to produce coke instead of residual fuel oil, or of so-called blowdown oil obtained when steaming the coking chamber of a cracking process after it has been filled with coke and before removing the latter.

Less desirable but also useful are high-boiling vapor phase cracked or other highly aromatic hydrocarbon distillates, such as extracts produced by extracting kerosenes, gas oils, etc., with selective solvents having preferential solvent power for aromatic hydrocarbons, providing such distillates are sufficiently aromatic and free of olefins, e. g. containing at least 50% of aromatics. To make these aromatic fractions free of sludge-forming propensities, sulfur and other impurities are often removed by treating the distillate with sulfuric acid, aluminum chloride, clays, or other treating agents.

The aromatic hydrocarbons discussed hereinbefore may be oxidized by one of several oxidation methods provided conditions are such as to suppress formation of hydrocarbon peroxides as much as possible. Thus we may oxidize with hydrogen peroxide, manganese dioxide, permanganates, chlorates, perchlorates, perborates, cro-mates, chromic acid, etc., preferably under conditions that will not cause ring cleavage and if desired in the presence of catalysts that tend to destroy organic peroxides.

Our preferred method consists of passing gaseous oxygen at atmospheric or higher pressures through the aromatic hydrocarbons at temperatures between 110° C. and 250° C. and preferably between 140° C. to 180° C. This temperature range is desirable, inasmuch as it permits fairly rapid oxidation under conditions at which peroxides are comparatively unstable with the result that an oxidized material is obtained, containing few if any peroxides.

The degree of oxidation may, at any point, be determined by either one of two convenient methods. The first method consists of withdrawing a sample and fractionally distilling it to determine the amount of unoxidized material boiling at the temperature of the original untreated aromatic hydrocarbons. The second method, applicable when oxidizing with free oxygen, consists of determining the total absorption of free oxygen, and collecting and measuring quantities of carbon dioxide and water evolved in the course of the oxidation, the amount of oxygen introduced into the hydrocarbons being calculated by difference. Thus the degree of oxidation may be expressed in percent of hydrocarbons oxidized or in percent of oxygen content of the oxidized hydrocarbons. The two methods of expressing the oxygen content can approximately be correlated by determining the average molecular weight of the hydrocarbons. Thus

$$\text{Per cent oxygen in hydrocarbons} = \frac{\text{Per cent oxidized hydrocarbons} \times 16}{\text{avg. mol. wt. of the hydrocarbons}}$$

The extent of oxidation is preferably such that about 5 to 50% of the hydrocarbon materials have been oxidized. If desired, however, lower or higher percentage of oxidized components are permissible. As already indicated, the peroxide content should be as low as possible, preferably less than about 1% of the oxidized hydrocarbons, although there is no critical limit for this amount. In general, the higher the peroxide content, the poorer are the anti-oxidant properties of the oxidized hydrocarbons.

The following example further illustrates our invention. In the table below are presented the induction periods of an uninhibited pure hydrocarbon oil, the hydrocarbon oil plus unoxidized secondary-amyl-naphthalene and alpha-methyl-naphthalene and the hydrocarbon oil plus identical percentages of the corresponding oxidized compounds which had been oxidized until they contained 1.7% and 1.2% by weight of absorbed oxygen or 20.7% and 10.8% of oxidized components respectively.

Table

| Hydro-carbon oil | Added aromatic                         | Time to absorb 400 ml. O <sub>2</sub> gm. mol. at 150° C. | Hours |
|------------------|----------------------------------------|-----------------------------------------------------------|-------|
| White oil        | +                                      |                                                           | 4     |
| White oil        | 10% sec. amyl-naphthalene              |                                                           | 1.6   |
| White oil        | 10% oxidized sec.-amyl-naphthalene     |                                                           | 14.0  |
| White oil        | 7.5% alpha-methyl-naphthalene          |                                                           | 2.0   |
| White oil        | 7.5% oxidized alpha-methyl-naphthalene |                                                           | 14.8  |

The preferred amounts of our oxidized aromatic fractions to be added to lubricating oils range from 2% to 10% by weight of the oil, although in most instances amounts within the range of .5% to 15% may be used.

Lubricating, transformer, or turbine oils containing our oxidized aromatic hydrocarbons de-

scribed before may be further improved by the addition of wax suppressors such as pour point or cloud point depressors, blooming agents, extreme pressure agents, anti-wear agents, corrosion inhibitors, and other compounding ingredients.

We claim as our invention:

1. A lubricating composition comprising a mineral hydrocarbon oil and dissolved therein a minor amount of a pre-oxidized aromatic hydrocarbon mixture obtained by oxidation under conditions to suppress ring cleavage and peroxide formation comprising passing gaseous oxygen through said aromatic hydrocarbon mixture at temperatures between about 110 and 250° C. and at least atmospheric pressure, said hydrocarbon mixture being free from olefins, and comprising predominantly aromatic hydrocarbons having at least 2 condensed rings, said oxidized mixture containing a substantial amount of oxidized components.

2. A lubricating composition comprising a mineral lubricating oil and dissolved therein a minor amount of a pre-oxidized aromatic hydrocarbon mixture obtained by oxidation under conditions to suppress ring cleavage and peroxide formation comprising passing gaseous oxygen through said aromatic hydrocarbon mixture at temperatures between about 110 and 250° C. and at least atmospheric pressure, said hydrocarbon mixture being free from olefins, and comprising predominantly alkyl substituted aromatic hydrocarbons having at least 2 condensed rings, said oxidized mixture containing a substantial amount of oxidized components.

3. A lubricating composition comprising a mineral lubricating oil and dissolved therein a minor amount of a pre-oxidized aromatic hydrocarbon mixture obtained by oxidation under conditions to suppress ring cleavage and peroxide formation comprising passing gaseous oxygen through said aromatic hydrocarbon mixture at temperatures between about 110 and 250° C. and at least atmospheric pressure, said hydrocarbon mixture being free from olefins and comprising predominantly alkyl substituted aromatic hydrocarbons having at least 2 condensed rings, said oxidized mixture containing between 5% and 50% by weight of oxidized components.

4. A lubricating composition comprising a mineral lubricating oil and dissolved therein a minor amount of a pre-oxidized aromatic hydrocarbon mixture obtained by oxidation under conditions to suppress ring cleavage and peroxide formation comprising passing gaseous oxygen through said aromatic hydrocarbon mixture at temperatures between about 110 and 250° C. and at least atmospheric pressure, said hydrocarbon mixture being free from olefins and comprising predominantly alkyl substituted aromatic hydrocarbons having at least 2 condensed rings, said oxidized mixture containing between 10% and 20% by weight of oxidized components.

5. A lubricating oil composition comprising a mineral hydrocarbon oil and dissolved therein a minor amount of a pre-oxidized aromatic hydrocarbon mixture obtained by oxidation under conditions to suppress ring cleavage and peroxide formation comprising passing gaseous oxygen through said aromatic hydrocarbon mixture at temperatures between about 110 and 250° C. and at least atmospheric pressure, said hydrocarbon mixture being free from olefins, and comprising predominantly cracked high aromatic hydrocarbon distillate, said oxidized mixture con-

taining a substantial amount of oxidized components.

6. A lubricating oil composition comprising a mineral hydrocarbon oil and dissolved therein a minor amount of a pre-oxidized aromatic hydrocarbon mixture obtained by oxidation under conditions to suppress ring cleavage and peroxide formation comprising passing gaseous oxygen through said aromatic hydrocarbon mixture at temperatures between about 110 and 250° C. and at at least atmospheric pressure, said hydrocarbon mixture being free from olefins, and comprising predominantly alkyl naphthylene, said oxidizing mixture containing a substantial amount of oxidizing components.

7. A lubricating oil composition comprising a mineral hydrocarbon oil and dissolved therein a minor amount of a pre-oxidized aromatic hydrocarbon mixture obtained by oxidation under conditions to suppress ring cleavage and peroxide formation comprising passing gaseous oxygen through said aromatic hydrocarbon mixture at temperatures between about 110 and 250° C. and at at least atmospheric pressure, said hydrocarbon mixture being free from olefins and comprising predominantly methyl naphthylene, said oxidizing mixture containing a substantial amount of oxidizing components.

8. A composition relatively stable to oxidation comprising a refined relatively viscous mineral oil subject to deterioration by oxidation and dissolved therein a small amount of a pre-oxidized aromatic hydrocarbon mixture obtained by oxidation under conditions to suppress ring cleavage and peroxide formation comprising passing gas-

ous oxygen through said aromatic hydrocarbon mixture at temperatures between about 110 and 250° C. and at at least atmospheric pressure, said hydrocarbon mixture being free from olefins and comprising predominantly aromatic hydrocarbons having at least 2 condensed rings, said oxidized mixture containing a substantial amount of oxidized components.

9. The method of inhibiting the oxidation of 10 a mineral lubricating oil normally susceptible to deterioration by oxidation comprising passing gaseous oxygen through an aromatic hydrocarbon mixture at a temperature between about 110 and 250° C. and at at least atmospheric pressure 15 so as to suppress ring cleavage and formations of peroxides, said hydrocarbon mixture being free from olefins and comprising predominantly aromatic hydrocarbons having at least 2 condensed rings, and adding a minor amount of the 20 resulting oxidized material to a larger amount of said lubricating oil.

10. The composition of claim 1 wherein said organic hydrocarbon mixture is oxidized at a temperature between about 140 and 180° C.

11. The composition of claim 3 in which the amount of the preoxidized mixture is from .5% to 15% by weight of the oil.

12. The composition of claim 3 in which the amount of the preoxidized mixture is from 2% to 10% by weight of the oil.

13. The composition of claim 1 wherein the peroxide content of the preoxidized hydrocarbon is less than about 1% of its oxidized components.

ROBERT G. LARSEN.  
FREDERIC A. ARMFIELD.